# EUROPEAN PATENT SPECIFICATION

(11) **EP 0 022 281 B1**
(45) Date of publication and mention of the grant of the patent: **14.09.1983**
(21) Application number: 80200511.6
(22) Date of filing: 30.05.1980
(51) Int. Cl.: C10M 3/28, C09K 15/18, C09K 15/20, C09K 15/24

(54) **Amino compounds and use of amino compounds as antioxydant in lubricating oils**
Aminoverbindungen und Verwendung von Aminoverbindungen als Antioxydationsmittel in Schmierölen
Composés amino et utilisation des composés amino comme antioxydant dans des huiles lubrifiantes

(30) Priority: 31.05.1979 US 43996
(43) Date of publication of application: 14.01.1981
(73) Proprietor: UNIROYAL, INC., New York, New York 10020 (US)
(72) Inventor: Bandlish, Baldev Kumar, Middlebury, New Haven Connecticut 06762 (US); Loveless, Frederick C., Cheshire, New Haven Connecticut 06410 (US); Nudenberg, Walter, Newtown, Fairfield CConnecticut 06470 (US)
(74) Representative: Kupecz, Arpad

## Description

Advanced automotive, aircraft and other industrial equipment require lubricating oils that are effective at elevated temperatures. Polyesters, polyolefins, polyglycols, polyphenyl ethers, phosphates, silicones, etc. have been used as suitable lubricating oils. These lubricating oils undergo oxidative degradation at elevated temperatures. Loss of lubricating properties due to oxidative breakdown of these oils may cause failure of a part, or parts, in contact with the oils. The prior art discloses the stabilization of lubricating oils using various amines including diphenyl- and substituted diphenylamines, p-phenylenediamine and substituted naphthylamine. There appears to be no recognition of the use of secondary amines wherein one of the groups attached the amino nitrogen is an aromatic or substituted aromatic ring and the other group is an aliphatic carbon which in turn is attached to an aromatic or substituted aromatic ring.

U.S.-A-1,469,245 discloses N-(o-Hydroxybenzyl)-N'-phenyl-p-phenylene diamine as an anti- degradant for rubber. This compound belongs to the class of phenylene diamines which are known antioxidants. Furthermore, its use as a stabilizer for lubricating oils is neither disclosed in that patent, nor elsewhere.

U.S.-A-2,108,147 teaches a method for preparing secondary and tertiary amines including 1-anilino-1-phenylethane. Hickenbottom teaches a phenylamine compound designated as alpha- phenylethyl-p-toluidine; see Journal of the Chemical Society (1934) pages 319-322. Beilstein discloses a phenyl amine compound of the general formula wherein R can be phenyl; see Handbuch Der Organischen Chemie 4th Ed., Vol XII Pat. IV pages 2403-4. None of the aforegoing compounds are taught to be antioxidants.

It has surprisingly been found that certain amino compounds can effectively be used as antioxidants in lubricative oils. These amino compounds have the general formula wherein Y is: When Y is the moiety of formula (II), Z is H or C₁ to C₃ alkyl; and X and R₂ are each independently selected from the group consisting of hydrogen, C,-C₁₂ alkyl, C₁-C₁₂ alkoxy; C₁-C₁₈ carbalkoxy, halogen, or nitro and R₁ is hydrogen, C₁ C₁₂ alkyl, C₁-C₁₂ alkoxy, C₁-C₁₈ carbalkoxy, halogen, amino or nitro. When Y is the moiety of formula (III), R₁ and R₃ are each independently selected from the group of moieties set forth as R, above and R₂ is as previously defined; provided, however, R, and R₂ may not be simultaneously hydrogen when Z is hydrogen.

In its preferred embodiment the antioxidants of this invention are used in conjunction with a metal deactivator and a metal or metal salt. The preferred metal salts are oil soluble organic salts, e.g., metal napthenates.

This invention relates to a compound for the stabilizing lubricating oils against oxidation and sludge formation. In particular this invention relates to stabilizing such oils utilizing phenylated benzylamines or phenylated tetrahydro naphthylamines, which may be substituted or unsubstituted, either alone or in conjunction with a metal deactivator and a metal compound. This stabilizer system provides a surprisingly high degree of resistance to oxidative breakdown of lubricating oils as well as resulting in dramatic reductions in sludge formation. Certain of the phenylated benzylamines and phenylated tetrahydro naphthylamines used in the practice of this invention are novel compounds.

More specifically, this invention relates to antioxidants which are amino compounds having the general formula wherein Y is: When Y is the moiety of formula (II), Z and X are each independently selected from the group consisting of H or C, to C₃ alkyl; provided that both X and Z are not simultaneously H; R₂ is selected from the group consisting of hydrogen, C₁-C₁₂ alkyl, C₁-C₁₂ alkoxy, C₁-C₁₈ carbalkoxy, p-acetyl, alpha-anilinoethyl, halogen, or nitro; and R₁ is hydrogen, C₁-C2 alkyl, C₁-C₁₂ alkoxy, C₂ C₁₈ carbalkoxy, halogen or nitro; and when Y is the moiety of formula III, R₁ and R₃ are each independently selected from the group consisting of hydrogen, C₁-C₁₂ alkyl, C₁-C₁₂ alkoxy, C₁-C₁₈ carbalkoxy, halogen, amino or nitro; and R₂ is hydrogen.

The compounds of the invention as defined above are novel compounds, provided that when Y is the moiety of formula (II), X is methyl and both Z and R₂ are hydrogen, R₁ is not p-methoxy. The compound N-(a/pha-methyl benzyl)-p-methoxyaniline has been disclosed in Chemical Abstracts, Vol. 63, 63, No. 4, August 16, 1965, abstract 4191 C, but no use as an antioxidant in lubricating oils is indicated in this reference.

Illustrative non-limiting examples of the novel antioxidants of this invention are
N-(alpha-methyl-p-octylbenzyl)aniline;
N-(alpha-methyl-p-nonylbenzyl)aniline;
N-(alpha-methyl benzyl)-p-nonylaniline;
N-(alpha-methyl benzyl)-p-dodecylaniline;
N-(alpha-methyl benzyl)-m-methoxyaniline;
N-(alpha-methyl benzyl)-o-methoxyaniline;
N-(alpha-methyl benzyl)-m-carbethoxyaniline;
N-(alpha-methyl benzyl)-o-carbethoxyaniline;
N-(alpha-methyl benzyl)-p-chloroaniline;
N-(alpha-methyl benzyl)-m-chloroaniline;
N-(alpha-methyl benzyl)-o-chloroaniline;
N-(alpha, alpha-dimethylbenzyl)aniline
1-(p-dodecylanilino)-1,2,3,4-tetrahydronaphthalene;
1-(p-carbethoxyanilino)-1,2,3,4-tetrahydronaphthalene;
N-(p-acetyl-alpha-methyl benzyl)aniline; and
1,4-bis-( 1-anilinoethyl)benzene.

The preferred antioxidants of this invention are
N-(alpha-methyl p-octylbenzyl)aniline and
N-(alpha-methyl benzyl)-p-nonylaniline.

Addition of the amines described above to lubricating oils imparts an unexpectedly high degree of resistance to oxidative breakdown.

The amines of this invention are useful in stabilizing a wide range of lubricating oils including polyester oils, mineral oils and synthetic hydrocarbon oils. The stabilizer system of this invention is particularly effective for use in polyolester lubricating oils.

The polylolester lubricating oils for which the stabilizer systems of this invention are suitable are synthetic lubricants based upon one or more organic carboxylic acid esters. Illustrative examples of such oils are diesters such as dioctyl sebacate or dinonyl adipate prepared by the reaction of a dibasic acid and a monohydric alcohol; triesters such as trimethylolpropane tripelogonate or trimethylolpropane tricaprilate prepared by the reaction of trimethylol propane and a monobasic acid; tetraesters such as pentaerythritol tetracaprilate prepared by the reaction of pentaerythritol and a monobasic acid; esters of trimethylolpropane or pentaerythritol prepared by reaction with mixtures of monobasic acids; or complex esters prepared by reacting mixtures of monobasic acids, dibasic acids and polyhdyric alcohols.

The synthetic hydrocarbon oils to which the stabilizer system of this system of this invention may be added are oligomers of alpha olefins. The preferred alpha olefins are Cₗ-C,₄ alpha-olefins. Normally, these hydrocarbon oils have a number of average molecular weight of about 280 to about 2,000; preferably about 350 to about 1,500. These lubricating oils have low unsaturation preferably having an iodine number of less than 3.

The term "antioxidant" when used in the specification and claims means the substituted phenylated amines and substituted tetrahydronaphthyiamines of this invention. The term "stabilizer system" as used in the specification means the aforegoing antioxidants in conjunction with a metal compound and a metal deactivator.

The metal may be present either as the free metal or a salt of a metal. The salt must be soluble in the lubricating oil and is preferably an organometallic salt.

The preferred salts include naphthenates, stearates, acetylacetonates, octoates, decanoates etc.

The metal deactivators useful in the practice of this invention are benzotriazole and benzotriazole derivatives. The benzotriazole derivative can be alkyl substituted or dialkyl amino alkyl substituted; preferably dialkyl amino alkyl substituted. Substitution is on the seconday nitrogen of the triangle. The alkyl group can be a C₁ to C₂₀ alkyl and each alkyl may be the same or different than the others. Preferably the alkyl groups are selected to give the benzotriazole derivative sufficient oil solubility to be incorporated into the lubricant in an effective amount e.g. C₆-C₁₂ alkyl. Typical of such compounds is Reomet 38 marketed by Ciba Geigy Co. The term "metal deactivator" as used in the specification and claims means a compound which when added to a lubricant will neutralize the catalytic effect of metals e.g. copper in promoting oxidation.

The various components of the antioxidant system which may be added in any order are used in the following amounts. The antioxidant of this invention is used in amounts varying from about 0.5 to about 5.0 parts by weight per 100 parts of the oil, preferably, about 1.0 to about 4.0 parts; more preferably 2.0 to 2.5 parts. The metal deactivators can be used in amounts of about 0.05 to about 1.0 part by weight per 100 parts of the oil, preferably, 0.1 to 0.3 part. Metal or metal salts are used in the amounts of about 1 to about 25 parts of metal by weight per million parts of the oil; preferably 2 to 10 parts. The preferred metal is copper.

The criteria used herein to evaluate the effectiveness of an antioxidant for lubricating oils are:
1) the amount of sludge produced,
2) the change in initial viscosity,
3) the change in neutralization number; and
4) the weight change of the test metals.

These criteria are determined after the oil containing the antioxidant system of this invention has been aged for 72 hours at 188°C (370°F) or after the oil containing the antioxidant system has been aged for 48 hours at 218°C (425°F).

The benefits of the antioxidants and stabilizers of this invention may be more readily appreciated by reference to the following examples. The term "polyester" as used in the specification and claims means a polyester prepared from a polyol by reacting the polyol with a stoichiometric equivalent of mono basic acids.

### Example 1

This example shows the unexpected ability of the antioxidant of the present invention to protect polyester based lubricating oils against oxidative degradation. The oil used was a commercially available polyolester fluid, Hercolube A (marketed by Hercules Inc.) and believed to be one prepared from pentaerythritol and a mixture of monocarboxylic acids, e.g., valeric acid and pelargonic acid.

Experiments were carried out in order to evaluate the effectiveness of the antioxidant. The oil sample used in runs B and C was prepared by adding N-(alpha-methylbenzyl) aniline in the amount set forth in Table I to 100 grams of the polyolester based oil. Sample D was similarly prepared containing phenyl alpha-naphthylamine, a commercially available stabilizer. The amounts used in each case are set forth in Table I.

Each of the samples was tested according to the following test procedures:
A 100 ml. sample having the compositions set forth in Table I is poured into a pyrex glass test cell and aged by inserting one end of a glass air delivery tube into the test cell while the remaining 25 ml. portions of each original oil sample is set aside and analyzed for neutralization number and Kinematic Viscosity in 10-^{s} m^{2.}s ' (centistokes) at 37.8°C (100°F). Around this glass air delivery tube immersed in the oil was placed from zero to four metal washers (Mg, Cu, Ag, and Fe) as identified in Table I. When more than one washer was used, they were separated from each other by glass spacers. These remained in the oil during the aging process and served to indicate the extent of corrosion of the oil oxidative decomposition products on the metal. The test cell was then fitted with a reflux condenser. The assembly was placed in a constant temperature aluminium block. An air hose was then attached to the other end of the air delivery tube and the air flow was adjusted so that five liters of air per hour was bubbled through the oil. This aging test was carried out for 48 hours at 218°C (425°F). After aging, the oil was filtered hot and the amount of sludge developed was collected and was determined and recorded in milligrams per 100 ml. of the oil. The filtered oil was then analyzed to determine changes in neutralization number and-Kinematic Viscosity at 37.8°C (100°F).

The neutralization number was determined by the color-indicator titration method according to ASTM Procedure D974-55T.

The Kinematic Viscosity was determined according to ASTM Procedure D445-53T.

The metal washers, which were weighed initially, were then carefully washed and weighed again to determine the weight change in grams.

The data in Table I dramatically show that when an amine such as N-(alpha-1 methylbenzyl aniline is added to a polyolester based lubricating oil the aged properties of oil Samples B and C are excellent as noted by very little change in the viscosity or neutralization number, very low sludge and essentially no weight change in the metals. The amine antioxidant clearly provides better all around protection than.a commercially available stabilizer (Sample D).

It should be noted that Sample C, wherein the test was conducted in the presence of copper, was slightly more deteroriated than Sample B, where no copper was present.

### Example II

This example demonstrates the effect of the addition of and changes in the levels of a metal deactivator such as Reomet-38, a benzotriazole derivative marketed by Ciba Geigy Co., on the stabilization of a polyolester based lubricating oil while the level of N-(alpha-methylbenzyl)aniline and copper are maintained constant. The samples were prepared as in EXAMPLE I.

The data in Table II shows that the addition of Reomet-38 at the levels tested is effective in controlling viscosity change, neutralization number change and sludge formation. The data further demonstrates that the addition of Reomet-38 dramatically controls the weight loss of the copper washer.

The data in Table II also shows that the addition of even low levels of the metal deactivator (samples B and C) provide better protection than when no deactivator is used (sample A).

### Example III

This example dramatically demonstrates that Reomet-38 cannot be included in the stabilizing system without incorporating copper either in the form of a soluble salt or in the form of a metal strip, washer, wire, etc. This example further shows how changes in the level of copper while maintaining constant N-(alpha-methylbenzyl)aniline and Reomet-38 levels effects stabilization. The samples were prepared as in EXAMPLE 1.

The data in Table III shows that a stabilizer system containing N-(alpha-methylbenzyl)aniline and Reomet-38 is ineffective in the absence of copper (Sample A, Table III) in decreasing the amounts of sludge, maintaining low viscosity, low neutralization number, and protecting the metal washers from oxidation. In the absence of copper, Reomet 38 functions as a pro-degradant. The data in Table III further shows that increasing amounts of copper above 10 ppm causes the stabilizer system to exhibit a decrease in its efficiency in controlling oxidative breakdown.

### Example IV

This example utilises data presented in Examples I, II and III to demonstrate the essence of the instant invention. See Table IV.

Clearly Sample II-D illustrates that when the amine, a metal deactivator and copper are present, the greatest protection is afforded to the oil. Sample I-B (amine but no copper), Sample I-C (amine and copper) and most dramatically Sample III-A (amine and metal deactivator but no copper) all show decreased protection when compared with II-D where all three components of the instant invention are present in the system.

### Example V

This example demonstrates how the stabilization of a polyolester based lubricating oil is affected by changes in the level of N-(a/pha-methylbenzyl)aniline while maintaining constant Reomet-38 level in the presence of a constant amount of copper metal. The samples were prepared as in EXAMPLE I, using the amounts of ingredients shown in Table V.

The data in Table V show that when a level of about 2.0 to 3.0 parts of N-(alpha- methylbenzyl)aniline was used together with 0.2 part of Reomet-38, a polyolester based lubricating oil is effectively stabilized. The preferred level of N-(alpha-methylbenzyl)aniline is shown to be from 2.0 to 2.5 parts.

It can be seen from the results of Table V that the level of the N-(a/pha-methylbenzyl)aniline is critical in producing polyolester based lubricating oils having outstanding aged physical properties while maintaining Reomet-38 at a constant level.

### Example VI

This example demonstrates how various substituted N-benzylanilines effect the stabilization of a polyolester based oil while maintaining a constant Reomet-38 level in the presence of a constant amount of copper metal.

Substituted N-benzylanilines were prepared by catalytic hydrogenation of the corresponding Schiffs bases. Five percent Pd/C was used as the catalyst and ethanol was used as the solvent for hydrogenating the Schiff's bases. Schiff's bases, in turn, were prepared by the reaction of the appropriate ketones and anilines in the presence of molecular sieves. About 40 grams of molecular sieves (Linde 5A) were added to 1.0 mole of ketone and 1.0 to 1.2 moles of aromatic amine in 200 ml. of benzene; see Kazuo Taguchi and F. H. Westheimer, J. ORG. CHEM. 36, 1570 (1971). The reaction mixture was refluxed with continuous removal of water until almost no free ketone could be detected in the reaction mixture by I.R. spectroscopy. The mixture was then filtered and the molecular sieves washed with benzene. The filtrate and washings were combined and evaporated to dryness under reduced pressure. The crude product was purified by either crystallization or by vacuum distillation.

The samples were prepared and tested as in EXAMPLE I using the amounts of ingredients as shown in Table VI.

The data in Table VI clearly show that substituted benzylanilines of this invention stabilize polyester based lubricating oils with respect to oxidative breakdown.

Substitution on the aromatic ring of the benzyl group seems to have little adverse effect.

### Example VII

A preferred embodiment of this invention involves alkylation in the benzyl ring and/or the aniline ring of the parent alpha-methyl benzyl aniline. This is beneficial in that it results in decreased volatility of the parent compound. Thus, such compounds as where R₂ can be H, or a C₁ to C₁₂ alkyl group and R₁ can be H or a C₄ to C₁₂ alkyl group; provided that R₁ and R₂ are not simultaneously both hydrogen. R₂ can be a C₁ to C₁₂ alkyl group which may or may not be branched. R₁ can be an alkyl group, preferably in the para-position or a tertiary alkyl group such as those derived from isobutylene, isobutylene dimer, isobutylene trimer, propylene trimer, alpha-methyl styrene and the like.

### Example VIII

This example shows how phenylated-alpha-tetralylamine affects the stabilization of a polyolester based lubricating oil.

The phenylated-alpha-tetralylamines were prepared according to the procedure described in EXAMPLE VI.

The samples were prepared as in Example I using the amounts of ingredients as shown in Table VIII.

The data in Table VIII shows that the addition of phenylated-alpha-tetralylamine, a metal deactivator and copper or a copper salt to a polyloester lubricating oil such as Hercolube A stabilizes the said oil against oxidative breakdown.

### Example IX

To 100 parts of polydecene synthetic hydrocarbon oil is added 2.0 parts of 1-(p-dodecylanilino)-1,2,3,4-tetrahydro-naphthalene and 0.5 part Reomet 38. Oxidative testing of the oil as described in Example II-E show that the above combination effectively protects synthetic hydrocarbon oils against oxidative breakdown.

### Example X

To 100 parts of mineral oil is added 2.0 parts of N-(alpha-methylbenzyl)-aniline and 0.5 parts Reomet 38 as in Example II.E. The resulting blend is found also to exhibit excellent antioxidant properties when an aging test is performed at elevated temperatures.

### Example XI

To 100 parts of polyoctene synthetic hydrocarbon oil is added 2.0 parts of N-(alpha- methylbenzyl)aniline and 0.5 parts Reomet 38 as in Example II.E. The resulting blend is found to exhibit excellent antioxidant properties when an aging test is performed at elevated temperatures.

### Example XII

To 100 parts of polydecene synthetic hydrocarbon oil is added 2.0 parts of N-(alpha- methylbenzyl)aniline and 0.5 parts Reomet 38 as in Example II.E. The resulting blend exhibits excellent anitoxidant properties when aging is performed at elevated temperatures.

### Example XIII

To 100 parts of a blend of 25 parts polyoctene and 75 parts trimethylol propane triheptanoate synthetic ester fluid is added 2.0 parts of N-(alpha-methylbenzyl) aniline and 0.5 parts Reomet 38 as in Example II.E. The resulting blend is found to exhibit excellent antioxidant properties when aging is performed at elevated temperatures.

### Example XIV

To 100 parts of a blend of 50 parts of polyoctene and 50 parts of trimethylol propane triheptanoate synthetic ester fluid is added 2.0 parts of N-(alpha-methylbenzyl)aniline and 0.5 parts Reomet 38 as in 'Example II.E. The resulting blend is found to exhibit excellent antioxidant properties when aging is performed at elevated temperatures.

### Example XV

A. A solution of p-nonyl acetophenone (90g), aniline (75g), Toluene (125ml) and pyridine (20ml) was refluxed with continuous removal of water. N-(alpha-methyl-p-nonyl benzylidene) aniline (XXX) was obtained by fractional distillation. XXX had a boiling point of 200-208°C at 10 Pa (0.075 millimeter).

Analysis calculated for C₂₃H₃₁N: C, 85.92; H, 9.72; N, 4.36. Found: C, 87.12; H, 10.07; N, 3.91.

B. N-alpha-methyl-p-nonyl benzylidene) aniline (XXX) (40g) prepared by the procedure described in Example XVI A was hydrogenated using 5% Pd/C as the catalyst and 95% ethanol as the solvent. N-(alpha-methyl-p-nonyl benzyl) aniline (XXXI) was obtained by fractional distillation. XXXI had a boiling point of 183°C at 20 Pa (0.15 millimeter).

### Example XVI

A solution of alpha, alpha-dimethyl benzyl alcohol (73g), aniline (150g), toluene (150ml) and p-toluene sulfonic acid (2.0g) was refluxed with continuous removal of water. N-(alpha, alpha, dimethyl benzyl) aniline (XXXII) was obtained by fractional distillation. XXXII had a boiling point of 121 °C at 9.3 Pa (0.07 millimeter).

Analysis calculated for C₁₅H₁₇N: C, 85.26; H, 8.11; N, 6.63. Found: C, 85.08; H, 7.97; N, 7.03.

### Example XVII

A. A solution of p-octylacetophenone (100g), aniline (85ml), pyridine (20ml) and toluene (200ml) was refluxed with the continuous removal of water. The product was a mixture of unreacted p-octyl acetophenone, aniline, pyridine and the Schiff's base. The desired N-(α-methyl-p-octyl-benzylidene) aniline (I) (65g) was separated from other components of the reaction mixture by fractional distillation. The desired product (I) had a boiling point of 192°C at 13.3 Pa (0.1 millimeter).

B. N-(α-methyl-p-octyl benzylidene) aniline (49g), prepared by the procedure described in Example IA was hydrogenated using 5% Pd/C as the catalyst and 95% ethanol as the solvent. N-(amethyl-p-octyl-benzyl)aniline (II) (40.5g) was obtained by fractional distillation. The desired product II had a boiling point of 173 to 178°C at 3.3 Pa (0.025 millimeter).

Analysis calculated for C₂₂H₃₁N: C, 85.43; H, 10.03; N, 4.53. Found: C, 86.46; H, 10.58; N, 4.54.

### Example XVIII

A. Nonyl benzene was prepared by alkylating benzene with mixed propylene trimer using Friedel Crafts reaction. Nonyl benzene was nitrated and reduced to give p-nonyl aniline. A solution of p-nonyl aniline (30g), acetophenone (60g), toluene (200ml) and pyridine (20mi) was refluxed with continuous removal of water. N-(a-methyl benzylidene)-p-nonyl aniline (III) was obtained by fractional distillation. III had a boiling point of 194°C at 6.6 Pa (0.05 millimeter).

B. N-(α-methyl benzylidene)-p-nonyl aniline (III) (16.5g) prepared by the procedure described in Example IIA was hydrogenated using 5% Pd/C as the catalyst and 95% ethanol as the solvent. N-(a-methyl benzyl)-p-nonyl aniline (IV) was obtained by fractional distillation. IV had a boiling point of 180-184°C at 3.3 Pa (0.025 millimeter).

### Example XIX

A. Solution of acetophenone (33.5g), p-dodecyl aniline (73g), benzene (50ml) was refluxed in the presence of molecular sieve (100g) with continuous removal of water. The crude product was purified by crystallizing it from ethanol to give N-(α-methyl benzylidene)-p-dodecyl aniline (V) (95g). V had a melting point of 47°C.

Analysis calculated for C₂₆H₃₇N: C, 85.89; H, 10.26; N, 3.85. Found: C, 85.96; H, 10.55; N, 4.13.

B. N-(α-methyl benzylidene)-p-dodecyl aniline (80g) prepared by the procedure described in Example IIIA was hydrogenated using 5% Pd/C as the catalyst and 95% ethanol as the 'solvent to give N-(α-methyl benzyl)-p-dodecyl aniline (VI). VI had a boiling point of 188°C at 4 Pa (0.03 millimeter)..

Analysis calculated for C₂₆H₃₉N: C, 85.42; H, 10.75; N, 3.83. Found: C, 85.49; H, 10.54; N, 4.01.

### Example XX

A. A solution of acetophenone (64ml), p-anisidine (65mg), benzene (100ml) was refluxed in the presence of molecular sieve (100g) with continuous removal of water. The crude product was purified by crystallizing it from ethanol to give N-(a-methyl benzylidene)-p-anisidine (VII) (50g). VII had a melting point of 81-82°C.

Analysis calculated for C₁₅H₁₅NO: C, 79.97; H, 6.71; N, 6.22. Found: C, 80.10; H, 6.78; N, 6.24.

B. N-(a-methyl benzylidene)-p-anisidine (VII) prepared by the procedure described in example IVA was hydrogenated using 5% Pd/C as the catalyst and 95% ethanol as the solvent to give N-(a-methyl benzyl)-p-anisidine (VIII). VIII had a melting point of 64°C.

Analysis calculated for C₁₅H₁₇NO: C, 79.26; H, 7.54; N, 6.16. Found: C, 79.98; H, 7.65; N, 6.22.

### Example XXI

A solution of acetophenone (120ml), o-anisidine (123ml), benzene (100ml) was refluxed with continuous removal of water. The crude product was purified by crystallizing it from ethanol to give N-(α-methyl benzylidene)-o-anisidine (IX) (90C). It was then hydrogenated using 5% Pd/C as the catalyst and 95% ethanol as the solvent to give N-(α-methyl benzyl)-o-anisidine (X). X had a boiling point of 117°C at 40 Pa (0.3 millimeter).

Analysis calculated for C₁₅H₁₇NO: C, 79.26; H, 7.54; N, 6.16. Found: C, 79.42; H, 7.72; N, 6.32.

### Example XXII

A. A solution of acetophenone (44ml), ethyl-p-aminobenzoate (60g), benzene (100ml) was refluxed in the presence of molecular sieve (1 00g) with continuous removal of water. The crude product was purified by crystallizing it from ethanol to give N-(α-methyl benzylidene)-p-carbethoxy aniline (XI). XI had a m.p. of 87°C.

Analysis calculated for C₁₇H₁₇NO₂: C, 76.38; H, 6.41; N, 5.24. Found: C, 76.59; H, 6.37; N, 5.33.

B. N-(α-methyl benzylidene)-p-carbethoxyaniline (XI) prepared by the procedure described in example XXIIA was hydrogenated using 5% Pd/C as the catalyst and 95% ethanol as the solvent to give N-(a-methyl benzyl)-p-carbethoxy aniline (XII). XII had a m.p. of 88°C.

Analysis calculated for C₁₇H₁₉NO₂: C, 76.38; H, 6.41; N, 5.24. Found: C, 76.58; H, 6.37; N, 5.33.

### Example XXIII

A. A solution of acetophenone (95ml), m-carbethoxy aniline (75ml), benzene (150ml) was refluxed in the presence of molecular sieve (50g) with continuous removal of water. The crude product was distilled under reduced pressure to give N-(a-methyl benzylidene)-m-carbethoxyaniline (XIII). XIII had a boiling point of 205°C at 13 Pa (0.1 millimeter).

Analysis calculated for C₁₇H₁₇NO₂; C, 76.38; H, 6.41; N, 5.24. Found: C, 75.96; H, 6.34; N, 5.32.

B. N-(α-methyl benzylidene)-m-carbethoxyaniline (27g) prepared by the procedure described in example VIIA was hydrogenated using 5% Pd/C as the catalyst and 95% ethanol as the solvent. N-(a-methyl benzyl m-carbethoxy aniline (XIV) was obtained by fractional distillation. XIV had a boiling point of 156°C at 13 Pa (0.1 millimeter).

Analysis calculated for C₁₇H₁₉NO₂: C, 76.38; H, 6.41; N, 5.24. Found: C, 75.60; H, 6.96; N, 5.36.

### Example XXIV

A. A solution of acetophenone (100ml), o-carbethoxyaniline (90ml), benzene (100ml) was refluxed in the presence of molecular sieve (40g) with continuous removal of water. N-(a-methyl benzylidene)-o-carbethoxyaniline (XV) was obtained by fractional distillation. XV had a boiling point of 123° at 13 Pa (0.1 millimeter).

Analysis calculated for C₁₇H₁₇NO₂: C, 76.38; H, 6.41; N, 5.24.

B. N-(a-methyl benzylidene)-o-carbethoxyaniline (13g) prepared by the procedure described in example XXVA was hydrogenated using 5% Pd/C as the catalyst and 95% ethanol as the solvent. N-(α-methyl benzyl)-o-carbethoxyaniline (XVI) (12g) was obtained by fractional distillation. XVI had a boiling point of 168°C at 185 Pa (1.4 millimeter).

Analysis calculated for C₁₇H₁₉NO₂: C, 76.38; H, 6.41; N, 5.24. Found: C, 76.50; H, 7.04; N, 5.28.

### Example XXV

A solution of acetophenone (132ml), p-chloroaniline (128g), benzene (150ml) was refluxed in the presence of molecular sieve (40g) with continuous removal of water. The crude product was crystallized from ethanol to give p-chloro-N-(a-methyl benzylidene) aniline (XVII). It was then hydrogenated using 5% Pd/C as the catalyst and 95% ethanol as the solvent. The crude product wa crystallized from ethanol and pet. ether to give p-chloro-N-(a-methyl benzyl)aniline (XVIII). XVIII had a melting point of 62°C.

Analysis calculated for C₁₄H₁₄CIN: C, 72.56; H, 6.08; N, 6.04. Found: C, 72.80; H, 6.19; N, 6.15.

### Example XXVI

A. A solution of acetophenone (130ml), m-chloroaniline (130ml) and benzene (200ml) was refluxed in the presence of molecular sieve (50g) with continuous removal of water. m-Chloro-N-(a-methyl benzylidene) aniline (XIX) was obtained by fractional distillation. XIX had a boiling point of 110°C at 3.3 Pa (0.025 millimeter).

Analysis calculated for C₁₄H₁₂CIN: C, 73.20; H, 5.26; N, 6.09. Found: C, 73.60; H, 5.19; N, 6.23.

B. m-Chloro-N-(α-methyl benzylidene) aniline (XIX) (24g) prepared by the procedure described in example XXVIIA was hydrogenated using 5% Pd/C as the catalyst and 95% ethanol as the solvent. m-Chloro-N-(a-methyl benzyl) aniline (XX) was obtained by fractional distillation. XX had a boiling point of 133°C at 20 Pa (0.15 millimeter).

Analysis calculated for C₁₄H₁₄CIN: C, 72.56; H, 6.08; N, 6.04. Found: C, 72.63; H, 6.16; N, 6.26.

### Example XXVII

A. A solution of acetophenone (130ml), 2-chloroaniline (130ml) and benzene (200ml) was refluxed in the presence of molecular sieve with continuous removal of water. o-Chloro-N-(a-methyl benzylidene) aniline (XXI) was obtained by fractional distillation. XXI had a boiling point of 111 °C at 13 Pa (0.1 millimeter).

Analysis calculated for C₁₄H₁₂CIN: C, 73.20; H, 5.26; N, 6.09. Found: C, 73.38; H, 5.20; N, 6.25.

B. o-Chloro-N-(a-methyl benzylidene) aniline (XXI) (15g) prepared by the procedure described in example XXVIIIA was hydrogenated using 5% Pd/C as the catalyst and 95% ethanol as the solvent. o-Chloro-N-(a-methyl benzyl) aniline (XXII) was obtained by fractional distillation. XXII had a boiling point of 134°C at 160 Pa (1.2 millimeter).

Analysis calculated for C₁₄H₁₄CIN: C, 72.56; H, 6.08; N, 6.04. Found: C, 73.38; H, 6.05; N, 6.23.

### Example XXVIII

A. A solution of p-diacetylbenzene (50g), aniline (80g) and benzene (120ml) was refluxed in the presence of molecular sieve (10g) with continuous removal of water. The crude product was crystallized from ethanol to give p-acetyl-N-(ce-methyl benzylidene) aniline (XXIII). XXIII had a melting point of 205°C.

B. p-Acetyl-N-(a-methylbenzylidene) aniline (XXIII) (30g) prepared by the procedure described in Example XXIXA was hydrogenated using 5% Pd/C as the catalyst and 95% ethanol as the solvent. p-Acetal-N-(α-methyl benzyl) aniline (XXIV) was obtained by fractional distillation. XXIV had a boiling point of 165°C at 13 Pa (0.1 millimeter).

Analysis calculated for C₁₆H₁₇NO: C, 80.30; H, 7.16; N, 5.85. Found: C, 80.00; H, 7.46; N, 5.50.

### Example XXIX

A mixture of p-acetyl-N-(α-methyl benzylidene) aniline (XXIII) (40g) prepared by the procedure described in example XXIXA and aniline (20ml) was hydrogenated using 5% Pd/C as the catalyst and 95% ethanol as the solvent. The crude product was crystallized from ethanol to give 1,4-Bis-(1-anilinoethyl) benzene (XXV). XXV had a melting point of 169-170°C.

### Example XXX

A. A solution of a-tetralone (50ml), dodecyl aniline (80g) and benzene (150ml) was refluxed in the presence of molecular sieve (100g) with continuous removal of water. The crude product was crystallized from ethanol to give N-(1,2,3,4-tetrahydronaphthylidene) aniline (XXVI). XXVI had a melting point of 53°C.

Analysis calculated for C₂₈H₃₉N: C, 86.31; H, 10.09; N, 3.59. Found: C, 87.91; H, 10.05; N, 3.76.

B. N-(1,2,3,4-tetrahydronaphthylidene) aniline (XXVI) (38g) prepared as described in example XXXIA was hydrogenated using 5% Pd/C as the catalyst and 95% ethanol as the solvent. The crude product was crystallized from ethanol to give 1-(p-dodecylanilino)-1,2,3,4-tetrahydronaphthalene (XXVII). XXVII had a melting point of 34°C.

Analysis calculated for C₂₈H₄₁N: C, 85.87; H, 10.55; N, 3.57. Found: C, 86.40; H, 10.69; N, 3.78.

### Example XXXI

A. A solution of a-tetralone (40mi), ethyl-p-aminobenzoate (42g) and benzene (100mi) was refluxed in the presence of molecular sieve (100g) with the continuous removal of water. The crude product was crystallized from ethanol to give N-(1,2,3,4-tetrahydronaphthylidene)-p-carbethoxyaniline (XXVIII). XXVIII had a m.p. of 108.5°C.

Analysis calculated for C₁₉H₁₉NO₂: C, 77.78; H, 6.58; N, 4.77. Found: C, 77.95; H, 6.42; N, 4.85.

B. N-(1,2,3,4-Tetrahydronaphthylidene)-p-carbethoxyaniline (XXVIII) (30g) prepared by the procedure described in example XXXIIA was hydrogenated using 5% Pd/C as the catalyst and 95% ethanol to give 1-(p-carbethoxy-anilino)-1,2,3,4-tetahydronaphthalene (XXIX). XXIX had a melting point of 34°C.

Analysis calculated for C₁₉H₂₁NO₂: C, 77.26; H, 7.17; N, 4.74. Found: C, 77.84; H, 7.27; N, 4.92.

## Claims

1. An antioxidant having the general formula wherein Y is wherein when Y is the moiety of formula (II), Z and X are each H or C₁ or C₃ alkyl provided that both X and Z are not simultaneously H; R₂ is selected from the group consisting of hydrogen, C₂-C₁₂ alkyl, C₂-C₁₂ alkoxy, C₂-C₁₈ carbalkoxy, p-acetyl, alpha-anilinoethyl, halogen or nitro; and R₁ is hydrogen, C₁-C₁₂ alkyl, C₁-C₁₂ alkoxy, C₂-C₁₈ carbalkoxy, halogen or nitro, provided that when X is methyl and both Z and R₂ are hydrogen R₁ is not p-methoxy; and when Y is the moiety of formula III, R₁ and R₃ are each independently selected from the group consisting of hydrogen, C₁-C₁₂ alkyl, C₁-C₁₂ alkoxy, C₂―C₁₈ carbalkoxy, halogen, amino or nitro; and R₂ is hydrogen; provided, however, R, and R₂ may not be, simultaneously, hydrogen when either Z or X is hydrogen.

2. The antioxidant according to claim 1 wherein Y is the moiety of formula (II).

3. The antioxidant according to claim 2 wherein R₁ and Z are hydrogen; X is methyl and R₂ is p-C₈H_{17,} p-C₉H₁₉, p-CH₃CO, or C₆H₅NH―CH(CH₃).

4. The antioxidant according to claim 2 wherein R₂ and Z are hydrogen; X is methyl and R₁ is p-C₉H_{19,} p-C₁₂H_{25,} m-OCH₃, o-OCH₃, m-COOC₂H_{5,} o-COOC₂H₅, p-CI, m-CI, or o-CI.

5. The antioxidant according to claim 2 wherein R₁ and R₂ are H and X and Z are methyl.

6. The antioxidant according to claim 1 where Y is the moiety of formula (III).

7. The antioxidant according to claim 6 wherein R₂ and R₃ are H and R₁ is p-C₁₂H₂₅ or p-COOC₂H₅.

8. The antioxidant according to claim 1 wherein the antioxidant is N-(alpha-methyl-p-octylbenzyl)aniline; N-(alpha-methyl-p-nonylbenzyl)aniline; or N-(p-acetyl-alpha-methyl benzyl)aniline.

9. The antioxidant according to claim 1 wherein the antioxidant is N-(alpha-methyl benzyl)-p-nonylaniline; N-(alpha-methyl benzyl)-p-dodecylaniline; N-(alpha-methyl benzyl)-m-methoxyaniline; N-(alpha-methyl benzyl)-o-methoxyaniline; N-(alpha-methyl benzyl)-m-carbethoxyaniline; N-(alpha-methyl benzyl)-o-carbethoxyaniline; N-(a/pha-methyl benzyl)-p-chloroaniline; N-(alpha-methyl benzyl)-m-chloroaniline; or N-(alpha-methyl benzyl)-o-chloroaniline.

10. The antioxidant according to claim 1 wherein the antioxidant is N-(alpha, alphadimethylbenzyl)aniline.

11. The antioxidant according to claim 1 wherein the antioxidant is 1-(p-dodecylanilino)-1,2,3,4-tetrahydronaphthalene; or 1-(p-carbethoxyanilino)-1,2,3,4-tetrahydronaphthalene.

12. The antioxidant according to claim 1 wherein the antioxidant is 1,4-bis-(1-anilinoethyl)benzene.

13. The antioxidant according to claims 8 or 9 wherein the antioxidant is N-(a/pha-methyl-p-octylbenzyl)aniline; or N-(a/pha-methyl benzyl)-p-nonylaniline.

14. The use in lubricating oils of an antioxidant having the general formula wherein Y is wherein when Y is the moiety of formula (II), Z is H or C₁ to C₃ alkyl; X and R₂ are each independently selected from the group consisting of hydrogen, C₁-C₁₂ alkyl, C₁-C₁₂ alkoxy, C₂-C₁₈ carbalkoxy, halogen or nitro; and R, is hydrogen, C₁-C₁₂ alkyl, C₁-C₁₂ alkoxy, C₂-C₁₈ carbalkoxy, halogen, amino or nitro; and when Y is the moiety of formula III, R₁ and R₃ are each independently selected from the group consisting of hydrogen, C₁-C₁₂ alkyl, C₁-C₁₂ alkoxy, C₂C₁₈' carbalkoxy, halogen, amino, or nitro; and R₂ is as previously defined; provided, however, R₁ and R₂ may not be, simultaneously, hydrogen when Z is hydrogen.

## Patentansprüche

1. Antioxidationsmittel der allgemeinen Formel worin Y ist, wobei in dem Fall, daß es sich bei Y um den Rest mit der Formel (II) handelt, Z und X jeweils H oder eine C₁- bis C₃₋Alkylgruppe bedeuten, wobei jedoch Z und X nicht gleichzeitig H bedeuten können, R₂ aus dem Wasserstoffatom, C₂- bis C₁₂-Alkylgruppen, C₁- bis C₁₂₋Alkoxygruppen, C₂- bis C₁₈-Carbalkoxygruppen, der p-Acetylgruppe, der a-Anilinoethylgruppe, Halogenatomen oder der Nitrogruppe ausgewählt ist und R₁ ein Wasserstoffatom, eine C₁- bis C₁₂-Alkylgruppe, eine C₁- bis C₁₂-Alkoxygruppe, eine C₂- bis C₁₈ Carbalkoxygruppe, eine Halogenatom oder eine Nitrogruppe bedeutet, wobei vorausgesetzt ist, daß R₁ keine p-Methoxygruppe bedeutet, wenn X eine Methylgruppe ist und Z und R₂ Wasserstoffatome sind, und in dem Fall, daß es sich bei Y um den Rest mit der Formel (III) handelt, R₁ und R₃ jeweils unabhängig voneinander aus dem Wasserstoffatom, C₁- bis C₁₂-Alkylgruppen, C₁- bis C₁₂-Alkoxygruppen, C₂- bis C₁₈-Carbaikoxygruppen, Halogenatomen, der Aminogruppe oder der Nitrogruppe ausgewählt sind und R₂ ein Wasserstoffatom bedeutet, wobei jedoch R_{I} und R₂ nicht gleichzeitig Wasserstoffatome sein können, wenn entweder Z oder X ein Wasserstoffatom bedeutet.

2. Antioxidationsmittel nach Anspruch 1, worin Y der Rest mit der Formel (II) ist.

3. Antioxidationsmittel nach Anspruch 2, worin R, und Z Wasserstoffatome sind, X eine Methylgruppe bedeutet und R₂ p-C₈H₁₇, p-C₉H₁₉, p-CH₃CO oder C₆H₅NH-CH(CH₃) ist.

4. Antioxidationsmittel nach Anspruch 2, worin R₂ und Z Wasserstoffatome sind, X eine Methylgruppe bedeutet und R₁ p-C₉H₁₉, p-C₁₂H₂₅, m-OCH₃, o-OCH₃, m-COOC₂H₅, o-COOC₂H₅, p-CI, m-CI oder o-CI ist.

5. Antioxidationsmittel nach Anspruch 2, worin R₁ und R₂ H bedeuten und X und Z Methylgruppen sind.

6. Antioxidationsmittel nach Anspruch 1, worin Y der Rest mit der Formel (III) ist.

7. Antioxidationsmittel nach Anspruch 6, worin R₂ und R₃ H bedeuten und R₁ p-C₁₂H₂₅ oder p-COOC₂H₅ ist.

8. Antioxidationsmittel nach Anspruch 1, bei dem es sich um N-(a-Methyl-p-octylbenzyl)-anilin, N-(a-Methyl-p-nonylbenzyl)-anilin oder N-(p-Acetyl-a-methylbenzyl)-anilin handelt.

9. Antioxidationsmittel nach Anspruch 1, bei dem es sich um N-(α-Methylbenzyl)-p-nonylanilin, N-(α-Methylbenzyl)-p-dodecylanilin, N-(α-Methylbenzyl)-m-methoxyanilin, N-(α-Methylbenzyl)-o-methoxyanilin, N-(α-Methylbenzyl)-m-carbethoxyanilin, N-(α-Methylbenzyl)-o-carbethoxyanilin, N-(a-Methylbenzyl)-p-chloranilin, N-(α-Methylbenzyl)-m-chloranilin oder N-(α-Methylbenzyl)-o-chloranilin handelt.

10. Antioxidationsmittel nach Anspruch 1, bei dem es sich um N-(α,α-Dimethylbenzyl)-anilin handelt.

11. Antioxidationsmittel nach Anspruch 1, bei dem es sich um 1-(p-Dodecylanilino)-1,2,3,4-tetrahydronaphthalin oder 1-(p-Carbethoxyanilino)-1,2,3,4-tetrahydronaphthalin handelt.

12. Antioxidationsmittel nach Anspruch 1, bei dem es sich um 1,4-Bis(1-anilinoethyl)-benzol handelt.

13. Antioxidationsmittel nach Anspruch 8 oder 9, bei dem es sich um N-(α-Methyl-p-octylbenzyl)-anilin oder N-(a-Methylbenzyl)-p-nonylanilin handelt.

14. Verwendung in Schmierölen eines Antioxidationsmittels der allgemeinen Formel worin Y ist, wobei in dem Fall, daß es sich bei Y um den Rest mit der Formel (II) handelt, Z H oder eine C₁- bis C₃₋Alkylgruppe bedeutet, X und R₂ jeweils unabhängig voneinander aus dem Wasserstoffatom, C₁- bis C₁₂-Alkylgruppen, C₁- bis C₁₂-Alkoxygruppen, C₂- bis C₁₈-Carbalkoxygruppen, Halogenatomen oder der Nitrogruppe ausgewählt sind und R, eine Wasserstoffatom, eine C₁- bis C₁₂-Alkylgruppe, eine C₁- bis C₁₂-Alkoxygruppe, eine C₂- bis C₁₈-Carbalkoxygruppe, ein Halogenatom, eine Aminogruppe oder eine Nitrogruppe bedeutet, und in dem Fall, daß es sich bei Y um den Rest mit der Formel (111) handelt, R₁ und R₃ jeweils unabhängig voneinander aus dem Wasserstoffatom, C₁- bis C₁₂-Alkylgruppen, C₁- bis C₁₂-Alkoxygruppen, C₂- bis C₁₈-Carbalkoxygruppen, Halogenatomen, der Aminogruppe oder der Nitrogruppe ausgewählt sind und R₂ die vorstehend definierte Bedeutung hat, wobei jedoch R₁ und R₂ nich gleichzeitig Wasserstoffatome sein können, wenn Z ein Wasserstoffatom bedeutet.

## Revendications

1. Anti-oxydant ayant pour formule générale dans laquelle Y est où quand Y est le fragment de formule (II), Z et X sont chacun H ou un alcoyle C₁ à C₃ à condition que X et Z ne soient pas simultanément H; R₂ est choisi dans le groupe consistant en hydrogène, alcoyle C₂―C₁₂, alcoxy C₁-C₁₂, carbalcoxy C₂―C₁₈, p-acétyle, alpha-anilinoéthyle, halogène ou nitro; et R₁ est de l'hydrogène, un alcoyle C₁-C₁₂ un alcoxy C₁-C₁₂, un carbalcoxy C₂-C₁₈, un halogène ou nitro, à condition que quand X est du méthyle et que Z et R₂ sont tous deux de l'hydrogène, R₁ ne soit pas p-méthoxy; et quand Y est le fragment de formule III, R₁ et R₃ sont chacun indépendamment choisis dans le groupe consistant en hydrogène, alcoyle C₁-C₁₂ alcoxy C₁-C₁₂, carbalcoxy C₂-C₁₈, halogène, amino ou nitro; et R₂ est de l'hydrogène; à condition cependant que R₁ et R₂ ne soient pas simultanément de l'hydrogène quand Z ou X est de l'hydrogène.

2. Anti-oxydant selon la revendication 1, où Y est le fragment de formule (II).

3. Anti-oxydant selon la revendication 2, où R₁ et Z sont de l'hydrogène; X est du méthyle et R, est p-C₈H₁₇, p-C₉H₁₉, p-CH₃CO ou C₆H₅NH-CH(CH₃).

4. Anti-oxydant selon la revendication 2, où R₂ et Z sont de l'hydrogène; X est du méthyle et R₁ est p-C₉H₁₉, p-C₁₂H₂₅, m-OCH3, o-OCH₃, m-COOC₂H₅, o-COOC₂H₅, p-CI, mCI, ou oCI.

5. Anti-oxydant selon la revendication 2, où R₁ et R₂ sont H et X et Z sont de méthyle.

6. Anti-oxydant selon la revendication 1, où Y est le fragment de formule (III).

7. Anti-oxydant selon la revendication 6, où R₂ et R₃ sont H et R₁ est p-C₁₂H₂₅ ou p-COOC₂H₅.

8. Anti-oxydant selon la revendication 1, où l'anti-oxydant est de la N-(alpha-méthyl-p-octylbenzyl)aniline; de la N-(alpha-méthyl-p-nonylbenzyl)aniline; ou de la N-(p-acétyl-alpha-méthyl- benzyl)aniline.

9. Anti-oxydant selon la revendication 1, où l'anti-oxydant est de la N-(alpha-méthylbenzyl)-p-nonylaniline; de la N-(alpha-méthylbenzyl)-p-dodécylaniline; de la N-(alpha-méthylbenzyl)-m-méthoxy- aniline; de la N-(alpha-méthylbenzyl)-o-méthoxyaniline; de la N-(alpha-méthylbenzyl)-m-carbéthoxy- aniline; de la N-(alpha-méthylbenzyl)-o-carbéthoxyaniline; de la N-(alpha-méthylbenzyl)-p-chloroaniline; de la N-(alpha-méthylbenzyl)-m-chloroaniline; ou de la N-(alpha-méthylbenzyl)-o-chloroaniline.

10. Anti-oxydant selon la revendication 1, où l'anti-oxydant est de la N-(alpha, alpha-diméthyl- benzyl)-aniline.

11. Anti-oxydant selon la revendication 1, où l'anti-oxydant est du 1-(p-dodécylanilino)-1,2,3,4-tétrahydronaphtalène; ou du 1-(p-carbéthoxyanilino)-1,2,3,4-tétrahydronaphtalène.

12. Anti-oxydant selon la revendication 1, où l'anti-oxydant est du 1,4-bis-(1-anilinoéthyl)benzène.

13. Anti-oxydant selon les revendications 8 ou 9, où l'anti-oxydant est de la N-(alpha-méthyl-p-octylbenzyl)-aniline ou de la N-(alpha-méthylbenzyl)-p-nonylaniline.

14. Utilisation, dans des huiles de lubrification, d'un anti-oxydant ayant le formule générale où Y est où quand Y est le fragment de formule (II), Z est H ou un alcoyle C₁ à C₃; X et R₂ sont chacun indépendamment choisis dans le groupe consistant en hydrogène, alcoyle C₁―C₁₂, alcoxy C₁―C₁₂, carbalcoxy C₂―C₁₈, halogène ou nitro; et R₁ est de l'hydrogène, un alcoyle C₁―C₁₂, un alcoxy C₁―C₁₂, un carbalcoxy C₂―C₁₈, un halogène, un amino ou nitro; et quand Y est le fragment de formule III, R, et R₃ sont chacun indépendamment choisis dans le groupe consistant en hydrogène, alcoyle C₁―C₁₂, alcoxy C₁―C₁₂, carbalcoxy C₂―C₁₈, halogène, amino ou nitro; et R₂ est tel que précédemment défini; à condition cependant que R, et R₂ ne soient pas simultanément de l'hydrogène quand Z est de l'hydrogène.
